

## UNITED STATES PATENT OFFICE

2,512,297

## MOTOR FUEL

Charles B. Biswell, Woodstown, and George Alvin Sayers, Penns Grove, N. J., assignors to E. I. du Pont de Nemours & Company, Wilmington, Del., a corporation of Delaware

No Drawing. Application October 27, 1948,  
Serial No. 56,922

17 Claims. (Cl. 44—69)

1

This invention relates to motor fuels and particularly to aviation motor fuels containing tetraethyl lead, ethylenedibromide and N,N'-di(secondary butyl)-p-phenylenediamine.

It has been found that N,N'-di(secondary butyl)-p-phenylenediamine is very effective to inhibit gum formation in cracked gasoline and to inhibit deterioration of tetraethyl lead added, or to be added, to motor fuels. When tetraethyl lead is added to a motor fuel, it is accompanied by at least an equimolecular amount of an organic halogen compound as a lead scavenger. In aviation motor fuels containing tetraethyl lead, the organic halogen compound is solely ethylenedibromide and is present in the proportion of substantially one mol for each mol of the tetraethyl lead.

Normally N,N'-di(secondary butyl)-p-phenylenediamine is quite stable and, when employed in a motor fuel in the absence of ethylenedibromide, it will, upon exposure to sunlight, slowly form a red product, apparently due to a photochemically induced oxidation, which color formation becomes objectionable in amount and intensity only after several days of exposure. Since, in practice, motor fuels are not subjected to such long exposures to sunlight and generally not more than 30 minutes, such color formation does not present a problem and there is no necessity for adding to the motor fuel any material to prevent such color formation.

When N,N'-di(secondary butyl)-p-phenylenediamine is employed in an aviation motor fuel in a concentration of at least 0.0014% by weight and the fuel also contains ethylene dibromide, a strong red colored product is formed rapidly upon exposure to sunlight. So long as the aviation fuel is maintained in the dark, it retains its original color over long periods of time. However, in practice, it is frequently necessary to expose it to sunlight for from about 10 to about 30 minutes and some times somewhat longer. When such fuel is exposed to sunlight, a rapid reaction takes place wherein ethylenedibromide and N,N'-di(secondary butyl)-p-phenylenediamine are consumed in stoichiometrical ratios to produce an intensely red product in sufficient quantities to alter the color of the motor fuel to an objectionable extent in from a few seconds to 10 minutes. The color of such red product is so intense that even traces thereof seriously alter the color of the fuel. Such results are not altered by the substantially complete elimination of oxygen, as by first sweeping the fuel with nitrogen and thereafter keeping it blanketed with nitrogen.

2

It is thus apparent that the red product so formed is a different product formed by a different reaction or series of reactions than the product formed by the slow oxidation of N,N'-di(secondary butyl)-p-phenylenediamine in the absence of ethylenedibromide.

The formation of the red colored product, in motor fuels containing N,N'-di(secondary butyl)-p-phenylenediamine and ethylenedibromide on exposure to sunlight, is particularly serious in aviation fuels. Aviation fuels are composed substantially wholly of saturated hydrocarbons, such as straight-run gasoline, isooctane, neohexane, reformed gasoline, hydroformed gasoline, polymer gasoline, alkylate and blends of two or more thereof, and usually contain tetraethyl lead and ethylenedibromide as the sole lead scavenger. Aviation fuels are manufactured to have different octane numbers, usually 91, 100 and 115 octane, and each motor is specially designed to operate with a fuel of a particular octane number and will not operate properly with a fuel of a different octane number and particularly a lower octane number. Accordingly, aviation fuels of different octane numbers are dyed different identifying colors, 91 octane fuel being dyed blue, 100 octane fuel being dyed green and 115 octane fuel being dyed purple. The formation of red products in such fuels changes their identifying colors; changing blue fuel to purple, changing green fuel to gray and then purple, and making purple fuel very much redder. This has caused the erroneous identification of aviation fuels resulting in the loss of aviation motors and endangering human life.

It is an object of our invention to provide aviation fuels containing tetraethyl lead, ethylenedibromide, N,N'-di(secondary butyl)-p-phenylenediamine and an organic nitrogenous base to prevent rapid change in color of the aviation fuel upon exposure to sunlight. Another object is to discharge color formed in an aviation fuel, containing tetraethyl lead, ethylenedibromide and N,N'-di(secondary butyl)-p-phenylenediamine, upon exposure to sunlight. A further object is to prevent change in color of aviation motor fuels containing tetraethyl lead, ethylenedibromide and N,N'-di(secondary butyl)-p-phenylenediamine. Other objects are to provide new compositions of matter and to advance the art. Still other objects will appear hereinafter.

The above and other objects may be accomplished in accordance with our invention which comprises adding to an aviation motor fuel, containing tetraethyl lead, ethylenedibromide and

N,N'-di(secondry butyl)-p-phenylenediamine, from about 0.25 mol to about 3 mols of an organic nitrogenous base for each mol of N,N'-di(secondry butyl)-p-phenylenediamine, the organic nitrogenous base being composed solely of carbon atoms, hydrogen atoms and at least one basic nitrogen atom, and said organic nitrogenous base having a dissociation constant of from about  $2 \times 10^{-3}$  to about  $1 \times 10^{-7}$ , boiling above 30° C. at atmospheric pressure and being free of multiple bonds other than those of a benzene ring. We have found that, when such amounts of such organic nitrogenous bases are added to such aviation fuels, they effectively prevent the formation of the intensely red products, ordinarily formed by such fuels upon exposure to sunlight, for the periods of time required for practical purposes and usually for about 30 minutes or more. Also, if the aviation fuel has become colored by exposure to sunlight before the organic nitrogenous base has been added thereto, the addition of an organic nitrogenous base of our invention will discharge such color and restore the original color of the fuel. In the later case, it will generally be desirable to add a larger amount of the organic nitrogenous base, e. g., an amount sufficient to discharge the color plus an amount sufficient to prevent further color change for the desired period.

Our invention is particularly adapted to the treatment of aviation fuels which are substantially saturated hydrocarbons, such as straight-run gasoline, iso-octane, neohexane, reformed gasoline, hydroformed gasoline, polymer gasoline, alkylate and blends of any two or more thereof.

The aviation fuel will contain from about 0.5 cc. to about 8 cc. of tetraethyl lead per gallon of fuel and, preferably, from about 2 cc. to about 5 cc. per gallon. The ethylenedibromide will be present in the aviation fuel in the proportion of from about 0.22 cc. to about 3.6 cc. per gallon of fuel and, preferably, from about 0.9 cc. to about 2.25 cc. per gallon. The ethylenedibromide will be the sole lead scavenger and will be present in an amount chemically equivalent to the tetraethyl lead.

The aviation fuel will contain N,N'-di(secondry butyl)-p-phenylenediamine in the proportion of from about 0.0014% to about 0.008% by weight (from about 0.038 to about 0.218 gram per gallon of fuel) and, preferably, from about 0.0018% to about 0.004% by weight (from about 0.049 to about 0.109 gram per gallon of fuel). Generally, the amount of N,N'-di(secondry butyl)-p-phenylenediamine employed will be dependent upon the amount of tetraethyl lead in the fuel, increasing with increasing amounts of tetraethyl lead, since the most important function of the N,N'-di(secondry butyl)-p-phenylenediamine is to prevent decomposition of the tetraethyl lead, generally indicated by the formation of a haze or a precipitate.

The organic nitrogenous bases which are to be used in accordance with our invention are those which have dissociation constants of from about  $2 \times 10^{-3}$  to about  $1 \times 10^{-7}$  and, preferably, those having dissociation constants of from about  $2 \times 10^{-3}$  to about  $1 \times 10^{-5}$ , and are composed solely of carbon atoms, hydrogen atoms and one or more basic nitrogen atoms. Also, such organic nitrogenous bases should be free of multiple bonds other than those of a benzene ring; i. e., except for the carbon atoms of a benzene ring, no two atoms should be bonded together by a double or a triple bond, such as C=C, C≡C, C≡N and

C≡N. Also, in order to avoid danger of evaporation of the organic base from the fuel, the organic nitrogenous bases should be those which boil at temperatures above 30° C. at atmospheric pressures. The organic nitrogenous bases include primary, secondary and tertiary amines and polyamines and the reduced heterocyclic nitrogen bases, such as piperidine. While the organic nitrogenous bases may contain aromatic groups, the preferred compounds are those which are aliphatic in character and are completely saturated, such as the alkyl amines, the alicyclic amines, the alkylene polyamines, and the reduced heterocyclic nitrogenous bases. Organic nitrogenous bases, which have been found to be highly effective for preventing the production of the intensely red product by ethylenedibromide and N,N'-di(secondry butyl)-p-phenylenediamine in a motor fuel on exposure to sunlight, are listed below, together with the dissociation constants of representative members thereof:

|    | Organic Bases             | Dissociation Constant 'K' |
|----|---------------------------|---------------------------|
| 30 | Monoisopropylamine        | $4.3 \times 10^{-4}$      |
|    | Mono-normal butylamine    | $4.1 \times 10^{-4}$      |
|    | Mono-secondry butylamine  | $3.6 \times 10^{-4}$      |
|    | Mono-isamylamine          | $4.0 \times 10^{-4}$      |
|    | Mono-normal heptylamine   |                           |
|    | Mono-normal octylamine    |                           |
|    | Mono dodecylamine         | $4.3 \times 10^{-4}$      |
|    | Mono stearylamine         |                           |
|    | Di-isopropylamine         |                           |
|    | Di-normal butylamine      |                           |
|    | Di-normal amylamine       |                           |
|    | Tri-normal butylamine     |                           |
|    | N,N-Dimethylethylamine    |                           |
|    | Cyclohexylamine           | $4.4 \times 10^{-4}$      |
|    | Benzylamine               | $2 \times 10^{-3}$        |
|    | 1,2-ethylenediamine       | $8.5 \times 10^{-5}$      |
|    | 1,2-propylenediamine      |                           |
|    | Diethylenetriamine        |                           |
|    | Triethylenetetramine      |                           |
|    | Tetraethylenepentamine    |                           |
|    | Dipropylenetriamine       |                           |
|    | N-phenylethylenediamine   |                           |
|    | Tetrabutylethylenediamine |                           |
|    | Piperidine                | $1.6 \times 10^{-3}$      |
|    | Pyrrolidine               |                           |
|    | Dipiperidyl               |                           |
|    | Morpholine                | $2 \times 10^{-6}$        |
|    | Alpha-pipercoline         | $9.6 \times 10^{-4}$      |

The amount of the organic nitrogenous base or bases employed will be dependent upon the amount of N,N'-di(secondry butyl)-p-phenylenediamine, and will fall within the range of from about 0.25 mol to about 3 mols for each mol of the N,N'-di(secondry butyl)-p-phenylenediamine and, preferably, from about 0.3 mol to about 2.5 mols. Since not all of the organic nitrogenous bases are equally effective, the amount employed will vary somewhat with the effectiveness of the organic nitrogenous base. Where the organic nitrogenous base contains a single basic nitrogen atom, it will be employed in the proportion of from about 0.5 mol to about 3 mols for each mol of N,N'-di(secondry butyl)-p-phenylenediamine and, preferably, from about 0.6 mol to about 2.5 mols. Where the organic nitrogenous base contains a plurality of basic nitrogen atoms, it will be employed in the proportion of from about 0.25 mol to about 2 mols for each mol of N,N'-di(secondry butyl)-p-phenylenediamine and, preferably, from about 0.3 mol to about 1.7 mols. Larger proportions of the organic nitrogenous bases may be used, but without advantage, and will generally be undesirable as constituting an unnecessary impurity in the fuel.

The organic nitrogenous bases may be added to the aviation fuel prior to the addition of the other ingredients, such as tetraethyl lead, ethyl-enedibromide and N,N'-di(secondry butyl)-p-

phenylenediamine, simultaneously with the addition of any one or more of such ingredients, or subsequently to the addition of such ingredients. They may even be added after the intensely red colored product has been formed in the fuel whereby they will discharge such red color.

The organic nitrogenous bases cannot be added to ethylenedibromide or a concentrated solution or mixture of ethylenedibromide, such as those consisting of tetraethyl lead and ethylenedibromide; N,N'-di(secondary butyl)-p-phenylenediamine and ethylenedibromide; and N,N'-di(secondary butyl)-p-phenylenediamine, tetraethyl lead and ethylenedibromide, as the organic nitrogenous base and ethylenedibromide combine under such conditions to form an ammonium salt which precipitates from such solutions and mixtures. Such salt does not prevent the rapid formation of the red product, when incorporated in fuel containing N,N'-di(secondary butyl)-p-phenylenediamine and ethylenedibromide with subsequent exposure of the motor fuel to sunlight. When such salt is added to motor fuel containing N,N'-di(secondary butyl)-p-phenylenediamine but no ethylenedibromide and the fuel is exposed to sunlight, the red product is formed in a few minutes but at a slower rate than when uncombined ethylenedibromide is present. Accordingly, it is necessary to add the organic nitrogenous bases to the motor fuel independently of the ethylenedibromide.

The organic nitrogenous bases must be used as such. Their salts are inoperable as will appear from the preceding paragraph and the following experiment. A motor fuel, containing N,N'-di(secondary butyl)-p-phenylenediamine, ethylenedibromide and an organic nitrogenous base of our invention, was exposed to sunlight for a period sufficient to produce an intense red color in the absence of the organic nitrogenous base. Thereafter, acids, e. g., acetic acid and hydrobromic acid, were added to samples of the motor fuel in an amount sufficient to neutralize the organic nitrogenous base, whereupon the intense red color was produced instantly.

In order to more clearly illustrate our invention, preferred modes of carrying the same into effect and advantageous results to be obtained thereby, the following examples are given:

#### EXAMPLE 1

Samples of an aviation fuel (containing 2 milliliters of tetraethyl lead, 0.9 milliliter of ethylenedibromide, 0.0075 gram of a blue gasoline dye and 0.098 gram of N,N'-di(secondary butyl)-p-phenylenediamine per gallon of fuel) were placed in clear glass sample bottles, 100 cc. fuel to each bottle. Except for a control sample, different organic nitrogenous bases were added to the separate samples of fuel in the proportions of 0.0005%, 0.0006%, 0.0007% and 0.001% by weight based on the fuel, corresponding to about 13.9%, 16.7%, 19.5% and 27.8% by weight, respectively, based on the N,N'-di(secondary butyl)-p-phenylenediamine. The samples were well mixed and immediately placed in direct sunlight together with the control sample. The untreated control sample turned from blue to purple within 2 minutes, whereas the samples, to which the organic nitrogenous bases were added, were much more resistant to color change. The organic nitrogenous bases employed, their concentrations in the fuel, the mol ratio (mols of organic nitrogenous base to each mol of N,N'-di(secondary butyl)-p-phenylenediamine), and the time in

minutes for the color to change from blue to purple are shown in the following Table I:

Table I

|    | Amine                | Per Cent Conc. | Mol Ratio | Time |
|----|----------------------|----------------|-----------|------|
| 5  | None                 |                |           |      |
|    | Isopropylamine       | 0.0006         | 0.626     | 2    |
|    | Do                   | 0.001          | 1.037     | >90  |
| 10 | n-Butylamine         | 0.0005         | 0.420     | 7    |
|    | Do                   | 0.0004         | 0.504     | >60  |
|    | Do                   | 0.001          | 0.843     | >90  |
|    | sec-Butylamine       | 0.0005         | 0.420     | 6    |
|    | Do                   | 0.0006         | 0.504     | 11   |
|    | Do                   | 0.001          | 0.843     | >90  |
| 15 | Isoamylamine         | 0.0005         | 0.352     | 6    |
|    | Do                   | 0.0006         | 0.423     | 20   |
|    | Do                   | 0.001          | 0.704     | >90  |
|    | Cyclohexylamine      | 0.0005         | 0.309     | 8    |
|    | Do                   | 0.0007         | 0.434     | 18   |
|    | Do                   | 0.001          | 0.618     | >90  |
|    | Triethylenetetramine | 0.0005         | 0.210     | 12   |
|    | Do                   | 0.0006         | 0.251     | 50   |
| 20 | Do                   | 0.0007         | 0.294     | >60  |
|    | Piperidine           | 0.0005         | 0.360     | 10   |
|    | Do                   | 0.0007         | 0.504     | >25  |
|    | Do                   | 0.001          | 0.722     | >90  |

#### EXAMPLE 2

25 A 100 cc. sample of aviation fuel (containing 2 cc. of tetraethyl lead, 0.9 cc. of ethylenedibromide, 0.015 gram of a green dye and 0.098 gram of N,N'-di(secondary butyl)-p-phenylenediamine per gallon of fuel) was treated with 0.0006% by weight of triethylenetetramine. This corresponds to about 16.7% by weight of triethylenetetramine based on the N,N'-di(secondary butyl)-p-phenylenediamine and a mol ratio of 0.251 to 30 1. The treated sample and an untreated sample of the same fuel were placed in direct sunlight. The untreated sample became dark gray in color within 5 minutes, and developed a distinct purple color within 10 minutes. The green color of the treated sample had not changed after 45 minutes of exposure.

#### EXAMPLE 3

35 A sample of 115 octane, aviation fuel (containing 45 a purple dye, 2 cc. tetraethyl lead, 0.9 cc. ethylenedibromide and 0.098 gram N,N'-di(secondary butyl)-p-phenylenediamine per gallon of fuel) was exposed to direct sunlight simultaneously with a sample of the same fuel to which had been added 0.0006% by weight of dipropylene-50 triamine (about 16.7% by weight of dipropylene-triamine based on the N,N'-di(secondary butyl)-p-phenylenediamine and a mol ratio of 0.314 to 55 1). After 5 minutes exposure, the untreated sample of fuel had become very much redder in color. The sample, containing the dipropylenetriamine, had not changed even after 45 minutes of exposure.

#### EXAMPLE 4

60 One gallon of iso-octane (containing 2 cc. tetraethyl lead, 0.9 cc. ethylenedibromide and 0.098 gram of N,N'-di(secondary butyl)-p-phenylenediamine) was divided into 100 cc. portions which were placed in clear glass sample bottles. Some of these portions were treated 65 with 0.001% by weight of organic nitrogenous bases (about 27.8% by weight based on the N,N'-di(secondary butyl)-p-phenylenediamine). These treated samples were then placed in direct 70 sunlight along with a control sample of the fuel to which no organic nitrogenous base had been added. The control sample turned distinctly pink within 10 seconds. None of the treated samples showed any color change after 60 minutes exposure. The organic nitrogenous bases

and the mols thereof for each mol of N,N'-di(secondary butyl)-p-phenylenediamine are shown in the following Table II:

Table II

| Base                    | Mols  |
|-------------------------|-------|
| Mono-n-heptylamine      | 0.532 |
| Mono-n-octylamine       | 0.475 |
| Pyrrolidine             | 0.863 |
| Dipiperidyl             | 0.365 |
| Morpholine              | 0.704 |
| 1,2-Propylenediamine    | 0.828 |
| 1,2-Ethylenediamine     | 1.020 |
| Diethylene triamine     | 0.595 |
| Tetraethylene pentamine | 0.324 |

## EXAMPLE 5

To 100 cc. portions of an aviation gasoline (containing 2 cc. tetraethyl lead, 0.9 cc. ethylenedibromide and 0.098 gram of N,N'-di(secondary butyl)-p-phenylenediamine per gallon of gasoline) were added organic nitrogenous bases in the proportion of 0.0032% by weight based on the fuel or about 89% by weight based on the N,N'-di(secondary butyl)-p-phenylenediamine. The treated samples, along with a control sample of the fuel to which no organic nitrogenous base had been added, were exposed to direct sunlight in clear glass containers. The control sample turned distinctly pink within 0.5 minute, whereas the treated samples showed no color change over the periods during which they were observed. The organic nitrogenous bases employed, the mols thereof for each mol of N,N'-di(secondary butyl)-p-phenylenediamine and the periods in minutes during which they were observed are shown in the following Table III:

Table III

| Base                       | Moles | Period |
|----------------------------|-------|--------|
| Dodecylamine               | 1.190 | 60     |
| Stearylamine               | 0.774 | 60     |
| Diisopropylamine           | 2.180 | 60     |
| Di-n-butylamine            | 1.710 | 60     |
| Benzylamine                | 2.060 | 40     |
| alpha-Picoline             | 2.230 | 40     |
| Tetrabutyl ethylenediamine | 0.774 | 40     |
| Phenylethylamine           | 1.610 | 40     |

## EXAMPLE 6

A sample of iso-octane (containing 4.6 cc. tetraethyl lead, 2.07 cc. ethylenedibromide, 0.0075 gram of a blue gasoline dye and 0.098 gram N,N'-di(secondary butyl)-p-phenylenediamine per gallon of iso-octane) changed from blue to purple in 1 minute when exposed to direct sunlight. Another sample of the same fuel was treated with 0.0012% by weight of n-butylamine, corresponding to 33.3% by weight based on the N,N'-di(secondary butyl)-p-phenylenediamine and a mol ratio of 1.007 to 1. The treated sample remained blue on exposure to direct sunlight for 120 minutes.

## EXAMPLE 7

A sample of iso-octane (containing 0.5 cc. tetraethyl lead, 0.225 cc. ethylenedibromide, 0.0075 gram of a blue gasoline dye and 0.098 gram N,N'-di(secondary butyl)-p-phenylenediamine per gallon of iso-octane) changed from blue to purple in 2.5 minutes when exposed to direct sunlight. Another sample of the same fuel was treated with 0.0012% by weight of n-butylamine, corresponding to 33.3% by weight based on the N,N'-di(secondary butyl)-p-phenylenediamine and a mol ratio of 1.007 to 1. The treated

sample remained blue on exposure to direct sunlight for 120 minutes.

## EXAMPLE 8

5 A sample of iso-octane (containing 4.6 cc. tetraethyl lead, 2.07 cc. ethylenedibromide, 0.0075 gram of a blue gasoline dye and 0.049 gram N,N'-di(secondary butyl)-p-phenylenediamine per gallon of iso-octane) changed from blue to purple in 5 minutes when exposed to direct sunlight. Another sample of the same fuel was treated with 0.0006% by weight of n-butylamine, corresponding to 33.3% by weight based on the N,N'-di(secondary butyl)-p-phenylenediamine and a mol ratio of 1.007 to 1. The treated sample remained blue on exposure to direct sunlight for 120 minutes.

## EXAMPLE 9

A gallon of iso-octane (containing 2 cc. tetraethyl lead, 0.9 cc. ethylenedibromide and 0.098 gram N,N'-di(secondary butyl)-p-phenylenediamine) was divided into 100 cc. portions which were placed in clear glass sample bottles. To two of the samples was added 0.001% and 0.002% by weight, respectively, of N-normal-butyl-p-aminophenol, corresponding to 27.8% and 55.6% by weight, respectively, based on the N,N'-di(secondary butyl)-p-phenylenediamine and mol ratios of 0.372 and 0.744, respectively, to 1. These samples were placed in direct sunlight along with a control sample of the same fuel to which no N-normal-butyl-p-aminophenol had been added. The control sample turned distinctly pink within 0.5 minute and the samples containing 0.001% and 0.002% of N-normal-butyl-p-aminophenol, turned pink in 0.75 minute and 1.0 minute, respectively.

When samples of the fuel of Example 9 were treated with 0.072% by weight of aniline, 0.0032% by weight of monomethylaniline, 0.0032% by weight of alpha-picoline, 0.001% by weight of quinoline, 0.072% by weight of pyridine and 0.072% by weight of N-methylpyrrole, respectively, it was found that neither aniline nor 45 N-methylpyrrole had any apparent effect to prevent or retard the color formation while the others gave results on the order of those obtained with N-normal-butyl-p-aminophenol. Dissociation constants "K" for representative amines of this group are; for aniline,

$$K=3.8 \times 10^{-10}$$

alpha-picoline,

$$K=4.0 \times 10^{-8}$$

55 pyridine,  $K=2.3 \times 10^{-9}$ ; and quinoline,

$$K=6.3 \times 10^{-10}$$

Example 9 and the paragraph which follows it 60 are included for comparative purposes and show that the dissociation constants and other limitations on the organic nitrogenous bases, to be used in accordance with our invention, are critical.

65 It will be understood that the preceding examples are given for illustrative purposes solely and that our invention is not to be limited to the specific embodiments disclosed therein, but we intend to claim our invention broadly as in the appended claims. It will be readily apparent to those skilled in the art that many variations and modifications can be made, particularly in the proportions of the various ingredients and in the organic nitrogenous bases employed within the 70 limits hereinbefore set forth without departing

from the spirit or scope of our invention. It will be particularly understood that mixtures of any two or more of such organic nitrogenous bases may be employed in place of any single such base.

It is well known that gum inhibitors in cracked gasoline tend to slowly deteriorate and form colored products which, however, become objectionable only after several days or weeks. Such deterioration is generally recognized to be an oxidation reaction and it has been found that various amines will inhibit such reaction.  $N,N'$  - di(secondary butyl) - p-phenylenediamine is also subject to such oxidative deterioration, but is more stable than most gum inhibitors so that the use of amines for preventing its oxidative deterioration is generally unnecessary. As shown by Example 9 and the paragraph immediately following it, the amines, which are most effective for inhibiting such oxidative deterioration, are not practically effective for preventing the formation of the red colored products by  $N,N'$  - di(secondary butyl) - p-phenylenediamine and ethylenedibromide in the presence of sunlight. Furthermore, the organic nitrogenous bases of our invention are relatively ineffective to inhibit the oxidative deterioration of  $N,N'$  - di(secondary butyl) - p-phenylenediamine and similar gum inhibitors. Accordingly, it is apparent that we are dealing with an entirely different problem involving a completely different reaction than the inhibition of oxidative deterioration of gum inhibitors. It is thus apparent that, by our invention, we have effectively solved a serious problem in the art in a novel manner and that our invention constitutes a new and valuable contribution to the art.

We claim:

1. A motor fuel consisting essentially of saturated hydrocarbon aviation fuel, from about 0.5 cc. to about 8 cc. of tetraethyl lead per gallon of aviation fuel, from about 0.22 cc. to about 3.6 cc. of ethylenedibromide per gallon of aviation fuel, from about 0.0014% to about 0.008% by weight of  $N,N'$  - di(secondary butyl) - p-phenylenediamine and from about 0.25 mol to about 3 mols of an organic nitrogenous base for each mol of  $N,N'$  - di(secondary butyl) - p-phenylenediamine, the organic nitrogenous base being composed solely of carbon atoms, hydrogen atoms and at least one basic nitrogen atom and having a dissociation constant of from about  $2 \times 10^{-3}$  to about  $1 \times 10^{-7}$  and boiling above 30° C. and being free of multiple bonds other than those of a benzene ring.

2. A motor fuel consisting essentially of saturated hydrocarbon aviation fuel, from about 0.5 cc. to about 8 cc. of tetraethyl lead per gallon of aviation fuel, from about 0.22 cc. to about 3.6 cc. of ethylenedibromide per gallon of aviation fuel, from about 0.0014% to about 0.008% by weight of  $N,N'$  - di(secondary butyl) - p-phenylenediamine and from about 0.25 mol to about 3 mols of a saturated organic nitrogenous base for each mol of  $N,N'$  - di(secondary butyl) - p-phenylenediamine, the organic nitrogenous base being composed solely of carbon atoms, hydrogen atoms and at least one basic nitrogen atom and having a dissociation constant of from about  $2 \times 10^{-3}$  to about  $1 \times 10^{-7}$  and boiling above 30° C.

3. A motor fuel consisting essentially of saturated hydrocarbon aviation fuel, from about 0.5 cc. to about 8 cc. of tetraethyl lead per gallon of aviation fuel, from about 0.22 cc. to about 3.6 cc. of ethylenedibromide per gallon of aviation fuel, from about 0.0014% to about 0.008% by weight of  $N,N'$  -

di(secondary butyl) - p-phenylenediamine and from about 0.5 mols to about 3 mols of a saturated organic nitrogenous base for each mol of  $N,N'$  - di(secondary butyl) - p-phenylenediamine, the organic nitrogenous base being composed solely of carbon atoms, hydrogen atoms and a single basic nitrogen atom and having a dissociation constant of from about  $2 \times 10^{-3}$  to about  $1 \times 10^{-7}$  and boiling above 30° C.

10. 4. A motor fuel consisting essentially of saturated hydrocarbon aviation fuel, from about 0.5 cc. to about 8 cc. of tetraethyl lead per gallon of aviation fuel, from about 0.22 cc. to about 3.6 cc. of ethylenedibromide per gallon of aviation fuel, from about 0.0014% to about 0.008% by weight of  $N,N'$  - di(secondary butyl) - p-phenylenediamine and from about 0.5 mol to about 3 mols of isopropylamine for each mol of  $N,N'$  - di(secondary butyl) - p-phenylenediamine.
15. 5. A motor fuel consisting essentially of saturated hydrocarbon aviation fuel, from about 0.5 cc. to about 8 cc. of tetraethyl lead per gallon of aviation fuel, from about 0.22 cc. to about 3.6 cc. of ethylene dibromide per gallon of aviation fuel, from about 0.0014% to about 0.008% by weight of  $N,N'$  - di(secondary butyl) - p-phenylenediamine and from about 0.5 mol to about 3 mols of piperidine for each mol of  $N,N'$  - di(secondary butyl) - p-phenylenediamine.
20. 6. A motor fuel consisting essentially of saturated hydrocarbon aviation fuel, from about 0.5 cc. to about 8 cc. of tetraethyl lead per gallon of aviation fuel, from about 0.22 cc. to about 3.6 cc. of ethylenedibromide per gallon of aviation fuel, from about 0.0014% to about 0.008% by weight of  $N,N'$  - di(secondary butyl) - p-phenylenediamine and from about 0.25 mol to about 2 mols of a saturated organic nitrogenous base for each mol of  $N,N'$  - di(secondary butyl) - p-phenylenediamine, the organic nitrogenous base being composed solely of carbon atoms, hydrogen atoms and a plurality of basic nitrogen atoms and having a dissociation constant of from about  $2 \times 10^{-3}$  to about  $1 \times 10^{-7}$  and boiling above 30° C.
25. 7. A motor fuel consisting essentially of saturated hydrocarbon aviation fuel, from about 0.5 cc. to about 8 cc. of tetraethyl lead per gallon of aviation fuel, from about 0.22 cc. to about 3.6 cc. of ethylenedibromide per gallon of aviation fuel, from about 0.0014% to about 0.008% by weight of  $N,N'$  - di(secondary butyl) - p-phenylenediamine and from about 0.25 mol to about 2 mols of diethylenetriamine for each mol of  $N,N'$  - di(secondary butyl) - p-phenylenediamine.
30. 8. A motor fuel consisting essentially of saturated hydrocarbon aviation fuel, from about 2 cc. to about 5 cc. of tetraethyl lead per gallon of aviation fuel, from about 0.9 cc. to about 2.25 cc. of ethylenedibromide per gallon of aviation fuel, from about 0.0018% to about 0.004% by weight of  $N,N'$  - di(secondary butyl) - p-phenylenediamine and from about 0.25 mol to about 3 mols of an organic nitrogenous base for each mol of  $N,N'$  - di(secondary butyl) - p-phenylenediamine, the organic nitrogenous base being composed solely of carbon atoms, hydrogen atoms, and at least one basic nitrogen atom and having a dissociation constant of from about  $2 \times 10^{-3}$  to about  $1 \times 10^{-7}$  and boiling above 30° C. and being free of multiple bonds other than those of a benzene ring.
35. 9. A motor fuel consisting essentially of saturated hydrocarbon aviation fuel, from about 2 cc. to about 5 cc. of tetraethyl lead per gallon of aviation fuel, from about 0.9 cc. to about 2.25 cc. of ethylenedibromide per gallon of aviation fuel,

from about 0.0018% to about 0.004% by weight of N,N'-di(secondary butyl)-p-phenylenediamine and an organic nitrogenous base composed solely of carbon atoms, hydrogen atoms and at least one basic nitrogen atom which has a dissociation constant of from about  $2 \times 10^{-3}$  to about  $1 \times 10^{-7}$  and boils above 30° C. and is free of multiple bonds other than those of a benzene ring, the organic nitrogenous base when it contains a single basic nitrogen atom being present in a proportion of from about 0.5 mol to about 3 mols for each mol of N,N'-di(secondary butyl)-p-phenylenediamine and when it contains a plurality of basic nitrogen atoms being present in a proportion of from about 0.25 to about 2 mols for each mol of N,N'-di(secondary butyl)-p-phenylenediamine.

10. A motor fuel consisting essentially of saturated hydrocarbon aviation fuel, from about 2 cc. to about 5 cc. of tetraethyl lead per gallon of aviation fuel, from about 0.9 cc. to about 2.25 cc. of ethylenedibromide per gallon of aviation fuel, from about 0.0018% to about 0.004% by weight of N,N'-di(secondary butyl)-p-phenylenediamine and a saturated organic nitrogenous base composed solely of carbon atoms, hydrogen atoms and at least one basic nitrogen atom which has a dissociation constant of from about  $2 \times 10^{-3}$  to about  $1 \times 10^{-5}$  and boils above 30° C., the organic nitrogenous base when it contains a single basic nitrogen atom being present in a proportion of from about 0.6 to about 2.5 mols for each mol of N,N'-di(secondary butyl)-p-phenylenediamine and when it contains a plurality of basic nitrogen atoms being present in a proportion of from about 0.3 to about 1.7 mols for each mol of N,N'-di(secondary butyl)-p-phenylenediamine.

11. A motor fuel consisting essentially of saturated hydrocarbon aviation fuel, from about 2 cc. to about 5 cc. of tetraethyl lead per gallon of aviation fuel, from about 0.9 cc. to about 2.25 cc. of ethylenedibromide per gallon of aviation fuel, from about 0.0018% to about 0.004% by weight of N,N'-di(secondary butyl)-p-phenylenediamine and from about 0.6 mol to about 2.5 mols of an organic nitrogenous base for each mol of N,N'-di(secondary butyl)-p-phenylenediamine, the organic nitrogenous base being composed solely of carbon atoms, hydrogen atoms and a single basic nitrogen atom and having a dissociation constant of from about  $2 \times 10^{-3}$  to about  $1 \times 10^{-5}$  and boiling above 30° C. and being free of multiple bonds other than those of a benzene ring.

12. A motor fuel consisting essentially of saturated hydrocarbon aviation fuel, from about 2 cc. to about 5 cc. of tetraethyl lead per gallon of aviation fuel, from about 0.9 cc. to about 2.25 cc. of ethylenedibromide per gallon of aviation fuel, from about 0.0018% to about 0.004% by weight of N,N'-di(secondary butyl)-p-phenylenediamine and from about 0.6 mol to about 2.5 mols of a saturated organic nitrogenous base for each mol of N,N'-di(secondary butyl)-p-phenylenediamine, the organic nitrogenous base being composed solely of carbon atoms, hydrogen atoms and a single basic nitrogen atom and having a dissociation constant of from about  $2 \times 10^{-3}$  to about  $1 \times 10^{-5}$  and boiling above 30° C.

13. A motor fuel consisting essentially of saturated hydrocarbon aviation fuel, from about 2 cc. to about 5 cc. of tetraethyl lead per gallon of aviation fuel, from about 0.9 cc. to about 2.25 cc. of ethylenedibromide per gallon of aviation fuel, from about 0.0018% to about 0.004% by weight of N,N'-di(secondary butyl)-p-phenylenediamine and from about 0.6 mol to about 2.5 mols of isopropylamine for each mol of N,N'-di(secondary butyl)-p-phenylenediamine.

14. A motor fuel consisting essentially of saturated hydrocarbon aviation fuel, from about 2 cc. to about 5 cc. of tetraethyl lead per gallon of aviation fuel, from about 0.9 cc. to about 2.25 cc. of ethylenedibromide per gallon of aviation fuel, from about 0.0018% to about 0.004% by weight of N,N'-di(secondary butyl)-p-phenylenediamine and from about 0.6 mol to about 2.5 mols of piperidine for each mol of N,N'-di(secondary butyl)-p-phenylenediamine.

15. A motor fuel consisting essentially of saturated hydrocarbon aviation fuel, from about 2 cc. to about 5 cc. of tetraethyl lead per gallon of aviation fuel, from about 0.9 cc. to about 2.25 cc. of ethylenedibromide per gallon of aviation fuel, from about 0.0018% to about 0.004% by weight of N,N'-di(secondary butyl)-p-phenylenediamine and from about 0.3 mol to about 1.7 mols of an organic nitrogenous base for each mol of N,N'-di(secondary butyl)-p-phenylenediamine, the organic nitrogenous base being composed solely of carbon atoms, hydrogen atoms and a plurality of basic nitrogen atoms and having a dissociation constant of from about  $2 \times 10^{-3}$  to about  $1 \times 10^{-5}$  and boiling above 30° C. and being free of multiple bonds other than those of a benzene ring.

16. A motor fuel consisting essentially of saturated hydrocarbon aviation fuel, from about 2 cc. to about 5 cc. of tetraethyl lead per gallon of aviation fuel, from about 0.9 cc. to about 2.25 cc. of ethylenedibromide per gallon of aviation fuel, from about 0.0018% to about 0.004% by weight of N,N'-di(secondary butyl)-p-phenylenediamine and from 0.3 mol to about 1.7 mols of a saturated organic nitrogenous base for each mol of N,N'-di(secondary butyl)-p-phenylenediamine, the organic nitrogenous base being composed solely of carbon atoms, hydrogen atoms and a plurality of basic nitrogen atoms and having a dissociation constant of from about  $2 \times 10^{-3}$  to about  $1 \times 10^{-5}$  and boiling above 30° C.

17. A motor fuel consisting essentially of saturated hydrocarbon aviation fuel, from about 2 cc. to about 5 cc. of tetraethyl lead per gallon of aviation fuel, from about 0.9 cc. to about 2.25 cc. of ethylenedibromide per gallon of aviation fuel, from about 0.0018% to about 0.004% by weight of N,N'-di(secondary butyl)-p-phenylenediamine and from about 0.3 mol to about 1.7 mols of diethylenetriamine for each mol of N,N'-di(secondary butyl)-p-phenylenediamine.

CHARLES B. BISWELL.  
GEORGE ALVIN SAYERS.